

Patented May 2, 1933

1,906,388

T. Scott

## UNITED STATES PATENT OFFICE

JAMES F. MCCLINTIC, OF DETROIT, MICHIGAN, ASSIGNOR TO GENERAL MOTORS RESEARCH CORPORATION, OF DETROIT, MICHIGAN, A CORPORATION OF DELAWARE

## SPRAY FOR COATING MOLDS

No Drawing.

Application filed May 31, 1929. Serial No. 367,630.

The object of this invention is to provide a coating for protecting the surfaces of molds against the erosive effects of the molten metal cast therein.

5 When molten metal is cast directly onto the surface of a green sand mold, the molten metal burns into the sand and a rough-surfaced casting, which is hard to clean, is produced. To the end of producing castings 10 having smooth surfaces, it has become the common practice to face the surfaces of green sand molds, which are to be exposed to the erosive effects of the molten metal, with a mixture of sea coal and molding sand to 15 prevent the molten metal from burning into the green sand. Although this practice has, to some extent, attained the desired objects, it has not been entirely successful and is more or less expensive and difficult to carry 20 out successfully.

I have discovered that if a finely powdered refractory is suspended in a suitable drying liquid or binder, which has been diluted to a suitable consistency with a rather highly 25 volatile liquid, a mixture is produced which may be applied to the surface of a mold with a spray gun or atomizer. On account of the rapid rate at which the diluent evaporates, which may be accelerated by spraying the 30 mixture on the mold while the latter is in a heated condition, there is practically no tendency for the mixture to run and the surface of the mold consequently becomes covered with a uniformly thick coating of finely di- 35 vided particles of refractory bound together by the drying liquid. To hasten the drying of the coating, the mold may be heated in a suitable oven.

40 Obviously, the operations described above may be, if necessary, repeated until a coating of the desired depth is obtained.

I have found that a mixture which consists of four (4) parts, by volume, of finely powdered plumbago suspended in a mixture 45 of two (2) parts, by volume, of core oil, which is a mixture of which linseed oil is the principal active ingredient and which ordinarily contains, in addition to the linseed oil, other active or inert ingredients such as rosin oil 50 and kerosene, and two (2) parts, by volume,

of gasoline is an eminently satisfactory spray for applying a protective coating to the surfaces of green sand molds. The proportions of the several ingredients may, of course, be varied to suit various conditions. The spray 55 may be applied directly to the surface of the green sand mold or may be applied to the surface of a coating of a mixture of sea coal and molding sand, which has previously been applied thereto. In the latter case, it is not necessary to use as thick a coating of the mixture of sea coal and molding sand as would otherwise be necessary.

Although the spray has been described with reference to its use in connection with 60 green sand molds, it is to be understood that it may, with equal facility and effectiveness, be used in connection with permanent molds or dry sand molds.

## I claim:

1. A spray for molds, which consists of four (4) parts, by volume, of finely powdered plumbago suspended in a mixture of two (2) parts, by volume, of core oil and two (2) parts, by volume, of gasoline.

2. A double coating for sand molds consisting of a layer of sea coal adhering to the mold surface and a superposed layer of powdered plumbago mixed with heavy oil and a highly volatile hydro carbon.

3. A coating for molds, which consists of a layer of sea coal adhering to the surface of the mold and a layer of plumbago and core oil superimposed on the layer of sea coal.

4. A preparation for coating molds which consist of plumbago, core oil and gasoline.

In testimony whereof I affix my signature.

JAMES F. MCCLINTIC.

90

95

100